

1

3,696,011

PROCESS FOR ELECTRODEPOSITING  
MANGANESE METAL

San-Cheng Lai, Oklahoma City, Okla., assignor to  
Kerr-McGee Chemical Corp., Oklahoma City, Okla.  
No Drawing. Filed Oct. 28, 1970, Ser. No. 84,936  
Int. Cl. C22d 1/24

U.S. CL. 204—105 M

3 Claims

ABSTRACT OF THE DISCLOSURE

A process for electrodepositing manganese metal wherein a selenium compound is added to a conventional manganese metal electrolyte to increase the current efficiency of the cell and a small quantity of sulfur dioxide is introduced to maintain the selenium compound in solution in the electrolyte.

BACKGROUND OF THE INVENTION

It is well known that in the electrodeposition of manganese metal, the addition of a small amount of sulfur dioxide to the electrolyte helps to prevent oxidation of the manganese ion in the solution and reduces the undesired formation of manganese dioxide on the anode. However, in commercial practice when sulfur dioxide is used as an additive, it has been found that current efficiencies in the cell are only about 60-65%.

In an article "Effect of Selenious Acid on the Electrodeposition of Manganese," by A. J. Rao, Y. D. P. Rao, and R. Vedaraman, published in the November—December 1966 (volume 4) issue of the Journal of Electrochemical Technology, it was reported that when selenious acid was used as an additive in place of sulfur dioxide in the electrodeposition of manganese metal that current efficiencies in excess of 90% could be obtained. Further, it has been reported that higher current densities can be used when selenium is used as the additive and that its use results in lower cell voltages when compared with conventional sulfate bath electrolytes wherein sulfur dioxide is used as the addition agent.

Summary of the invention

It now has been discovered that if a selenium compound is used as the sole additive, an orange precipitate or colloid or amorphous selenium metal forms in the electrolyte. This is disadvantageous, of course, because the selenium is thereby removed from the electrolyte solution and the advantages of its presence are lost. Further, costs are increased because of the necessity of having to replace the selenium which has precipitated out of solution.

Furthermore, the formation of the precipitate is disadvantageous because in the commercial electrodeposition of manganese metal, the electrolyte is introduced into the catholyte chamber of an electrolytic cell where the manganese is precipitated on the cathode. The catholyte then flows through a diaphragm into the anolyte compartment of the cell. The anolyte then is removed for purification before recycling to the catholyte compartment. When a selenium compound is used in such a process, it has been found that the selenium precipitate tends to deposit upon and plug the openings in the diaphragm of the cell, necessitating shutdown to either clean or replace the diaphragm.

The present invention is based upon the surprising discovery that a selenium precipitate does not form if a small amount of sulfur dioxide also is introduced into the electrolyte.

The selenium compound is added in amounts sufficient to obtain optimum current efficiencies and a deposit of

2

smooth, nodule-free manganese metal. Only enough sulfur dioxide is added to inhibit the formation of a selenium precipitate by maintaining the selenium compound substantially soluble in the electrolyte.

It is surprising that the sulfur dioxide inhibits the formation of a selenium precipitate in the electrolyte in view of the well-known analytical procedure in which sulfur dioxide is added to acidic test solutions to determine if selenium is present therein. If present, it forms a precipitate. In the present invention, smaller amounts of sulfur dioxide are used with the result that a selenium precipitate does not form.

DESCRIPTION OF THE PREFERRED EMBODIMENTS

The preferred electrolyte for the practice of this invention is ammonium sulfate containing a source of manganese. The best results have been obtained when the electrolyte was maintained at a pH of from about 7-8.5 and contained ammonium sulfate in an amount of from about 100 to 160 gm./liter and from about 11-45 gm./liter of manganese ion.

The selenium compounds which are suitable for use in the present invention are selenious acid ( $H_2SeO_3$ ) or other selenium compounds such as for example  $SeO_2$ ,  $SeO_3$ ,  $Na_2SeO_3$ ,  $(NH_4)_2SeO_3$ ,  $Na_2SeO_4$ ,  $(NH_4)_2SeO_4$  and the like. These compounds may be added to the electrolyte directly or fed in continuously as aqueous solutions. The concentration of selenium may be present in an amount of from 0.01-0.5 gm./liter. However, it is preferred that the concentration of selenium be from about 0.03 gm./liter to 0.1 gm./liter.

The sulfur dioxide may be added to the electrolyte by bubbling liquified or gaseous  $SO_2$  into the electrolyte. It also may be supplied by adding to the electrolyte compounds such as  $H_2SO_3$ ,  $Na_2SO_3$ ,  $(NH_4)_2SO_3$  and like which may be converted to  $SO_2$  in the electrolyte. The concentration of  $SO_2$  in the electrolyte should be sufficient to maintain the selenium compound in solution. Based on the quantity of selenium set forth herein, it has been found that the  $SO_2$  concentration should be maintained within the range of from about 0.01 to 0.1 gm./liter. However, the best results have thus far been obtained when the  $SO_2$  is present in an amount of from about 0.01 to 0.05 gm./liter.

EXAMPLE

To demonstrate the effectiveness of the present invention, a series of electrodepositions of manganese metal were carried out under the following conditions. The electrolyte had a:

pH—8.2

Temp.—35° C.

Current density—40 a.s.f.

The initial electrolyte consisted of:

|                | Gm./l. |
|----------------|--------|
| $Mn^{++}$      | 35     |
| $(NH_4)_2SO_4$ | 140    |

The results of these tests are shown in the following table.

From these tests it will be seen that the addition of  $SO_2$  to the electrolyte substantially reduces the precipitate formed in the catholyte. Further, it enhances the current efficiencies of the cell when used within the preferred range of from about .01 to .05 gm./liter. The presence of  $SO_2$  in amounts of 0.1 gm./liter and greater in the electrolyte result in the formation of a precipitate. The precipitate is believed to result from the reaction of the  $SO_2$  with the manganese salt solution to form manganese

sulfite in an amount in excess of its solubility in the electrolyte.

compound is selected from the group consisting of  $H_2SeO_3$ ,  $SeO_3$ ,  $(NH_4)_2SeO_3$ ,  $(NH_4)_2SeO_3$  and  $SeO_2$ .

## EXAMPLE

|                                                     | Se in the electrolyte, gm./liter |                     |                     |       |                   |                    |                    |      |                   |                    |                    |                    |                     |                     |       |
|-----------------------------------------------------|----------------------------------|---------------------|---------------------|-------|-------------------|--------------------|--------------------|------|-------------------|--------------------|--------------------|--------------------|---------------------|---------------------|-------|
|                                                     | 0.035                            |                     |                     |       | 0.07              |                    |                    |      | 0.1               |                    |                    |                    | 0.21                |                     |       |
| $SO_2$ in the electrolyte, gm./liter..              | 0                                | 0.01                | 0.05                | 0.1   | 0                 | 0.01               | 0.05               | 0.1  | 0.00              | 0.01               | 0.05               | 0                  | 0.001               | 0.05                | 0.1   |
| Precipitate formed in the catholyte, gm./liter..... | <sup>1</sup> 0.055               | <sup>2</sup> 0.0008 | <sup>2</sup> 0.0008 | 0.050 | <sup>1</sup> 0.08 | <sup>2</sup> 0.001 | <sup>2</sup> 0.001 | 0.06 | <sup>1</sup> 0.08 | <sup>2</sup> 0.001 | <sup>2</sup> 0.001 | <sup>1</sup> 0.095 | <sup>2</sup> 0.0075 | <sup>2</sup> 0.0082 | 0.074 |
| Current efficiency, percent.....                    | 89                               | 90.5                | 90                  | 89.4  | 92                | 93.8               | 94.5               | 90   | 92.0              | 93.8               | 94.5               | 90                 | 92                  | 92.4                | 89.5  |

<sup>1</sup> Orange precipitate appears in the catholyte.

<sup>2</sup> Clear catholyte.

What is claimed is:

1. In a process for electrodepositing manganese metal from an ammonium sulfate electrolyte containing manganese, the improvements which comprise introducing into said electrolyte a selenium compound in an amount sufficient to provide from about 0.01 to 0.5 gm./liter of selenium, based on the total volume of the electrolyte and effecting the deposition in the presence of sulfur dioxide in an amount within the range of from about 0.01 to 0.10 gm./liter to maintain the selenium compound in solution in said electrolyte.

2. The process of claim 1 wherein the selenium com-

15

3. The process of claim 1 wherein said selenium is present in an amount of about 0.1 gm. per liter of electrolyte and the sulfur dioxide is present in an amount of from about 0.01 to 0.05 gm. per liter of electrolyte.

## References Cited

20 "Effect of Selenious Acid on the Electrodeposition of Mn," by Rao et al., Electrochemical Technology, November-December 1966, vol. 4, pp. 536-539.

HOWARD S. WILLIAMS, Primary Examiner

R. L. ANDREWS, Assistant Examiner